

Nov. 25, 1969

W. EIRICH ET AL

3,480,261

PROCESS OF MIXING

Filed April 10, 1968

5 Sheets-Sheet 1



INVENTORS  
Wilhelm EIRICH  
Gustav EIRICH

Currie, Morris & Seftord  
ATTORNEYS

Nov. 25, 1969

W. EIRICH ET AL

3,480,261

PROCESS OF MIXING

Filed April 10, 1968

5 Sheets-Sheet 2



WATER/CEMENT RATIO

INVENTORS  
Wilhelm EIRICH  
Gustav EIRICH

Curtis, Morris & Safford  
ATTORNEYS

Nov. 25, 1969

W. EIRICH ET AL

3,480,261

PROCESS OF MIXING

Filed April 10, 1968

5 Sheets-Sheet 5

FIG. 3



INVENTORS  
Wilhelm EIRICH  
Gustav EIRICH

Curtis, Morris & Safford  
ATTORNEYS

Nov. 25, 1969

W. EIRICH ET AL

3,480,261

PROCESS OF MIXING

Filed April 10, 1968

5 Sheets-Sheet 4

FIG. 4



INVENTORS  
Wilhelm EIRICH  
Gustav EIRICH

Curtis, Monistett & Safford  
ATTORNEYS

Nov. 25, 1969

W. EIRICH ET AL

3,480,261

PROCESS OF MIXING

Filed April 10, 1968

5 Sheets-Sheet 5

FIG. 5



INVENTORS  
Wilhelm EIRICH  
Gustav EIRICH

Curtis, Monistafford  
ATTORNEYS

## 1

3,480,261

## PROCESS OF MIXING

Wilhelm Eirich, Bahnhofstr. 19, and Gustav Eirich, Wallerener Str. 41, both of Hardheim, Germany  
Filed Apr. 10, 1968, Ser. No. 720,043  
Claims priority, application Germany, Apr. 11, 1967,  
E 33,771  
Int. Cl. B28c 5/20, 7/02  
U.S. Cl. 259—148

8 Claims

## ABSTRACT OF THE DISCLOSURE

The disclosure relates to a process for the intensive mixing of the ingredients in the preparation of construction materials such as concrete, calcium silicate brick or the like and includes the steps of varying the speed of a mixing element and/or adding of water so as to maintain the energy input substantially constant at the rated capacity of the power operated drive. In one example the mixer is initially operated at a speed to produce the rated capacity and water is gradually added simultaneously with a gradual increase in speed to maintain operation at rated load. In another example all the remaining water required is added at one time and the speed of operation of the mixing element is correspondingly increased.

The present invention relates to a process for the intensive mixing of ingredients in the preparation of construction materials containing a binder, such as concrete, calcium silicate brick, or the like. The components of such materials are mixed in a mechanical mixer, preferably a disc or plate type mixer equipped with a high speed rotary mixing element, or with several mixing systems, at least one of which can be operated selectively at different speeds in several stages.

By such a method for intensive preparation of construction materials using a binder of lime or cement ground to the finest degree of subdivision, a high strength, particularly a high early setting strength, can be achieved and the amount of binder can be reduced in comparison to the conventional methods of preparation. Such a method of preparation also permits the largest possible amounts of energy to be introduced into the materials being mixed in a relatively short period of time, which results in a large output per unit weight of the materials being mixed. However, the driving efficiency for the mixers used for the preparation of construction materials cannot simply be increased at will. For instance, the energy absorption of the material being mixed is very strongly influenced by its consistency. In the region of a relatively low consistency (relatively high water/cement factor), the specific energy absorption of the mixture is, for example, so low that the desired advantage cannot be achieved. A further consideration of this kind of preparation is that a slight variation of the mixing procedure must be made for different concrete formulations. The binder content also influences the energy absorption of the mixture so that, for example, mixtures having a relatively low cement content produce an almost constant energy absorption whereas mixtures high in cement with an increasing proportion of water produce a sharp decrease in energy absorption.

The object of the invention is to provide a process for the preparation of construction materials in which a relatively large amount of energy can be introduced into a mixture in a short period of time and the binder content can be made more useful; and one in which the drive system for the mixer used in the preparation can be driven at its nominal or rated load during most of the entire mixing procedure so that a greater amount of energy

## 2

is employed than when a batch is prepared by conventional methods. Whereas, it has heretofore been assumed that when mixing materials, such as concrete, a uniform and homogeneous distribution of the components was decisive in achieving the highest possible value in the final product, the present invention resides in the discovery that by the further introduction of energy after the achievement of a completely homogenous mixture, the quality of the material, particularly its compressive strength, can be considerably increased, or if the same compressive strength is to be produced, a saving in binder of up to twenty percent can be achieved.

In accordance with the present invention the intensive preparation of materials such as concrete, with strength and/or saving in binder, is accomplished by mixing a binder and aggregate with quantity of thinner, such as water, and in such a manner that the mixer operates near its rated load and the mixing continued after the achievement of a homogenous mixture until further mixing work produces no further increase in the quality of the construction produced from the mixed product. The achievement of this ultimate condition is determined by a series of tests involving a variation in water/cement ratio, the duration of mixing, and the speed of the rotating element or elements of the mixing apparatus.

If, in a given case, as is particularly true in the case of concrete with a low water/cement factor, the added water required as determined by such tests, gives the consistency desired for further working, then the mixing procedure can be carried out in a single stage. In many cases, however, further addition of water after conclusion of the intensive mixing will be desirable or necessary.

According to one embodiment of the invention, cement and aggregate materials are initially combined with a fractional portion of the total amount of water required, and the mixing procedure is carried out during a period of operation of the mixing apparatus at a speed at which the maximum output of the drive for the mixer is introduced into the mixture. The remaining water is then introduced with a simultaneous increase in the speed of rotation of the mixing apparatus so that the mixer continues to operate at its nominal or rated load and the energy input into the mixed materials remains at the same value. By this kind of two-step process at different speeds, it is possible to introduce a large amount of energy into the mixed materials in a relatively short time so that an intensive reduction in particle size takes place while the mixing apparatus is simultaneously driven at its rated load. It is important that gel forming on the particles of cement be rubbed off, so that gel formation and hydration proceeds right to the core of the particle. The aggregate (stone and/or sand) functions in the process as a grinding medium and produces silica powder by abrasion. A further advantage is that the mixer can be driven during the preparation of the materials so that the drive motor runs at its nominal or rated capacity during the entire course of the work. The fractional amount of water used in the introductory step of the process, as well as the remaining water added in the second step carried out with an increased speed of the mixer, can be adapted to a variety of different concrete compositions so that the energy input into the mixture during the entire preparation of concrete remains at substantially the same value.

According to a further feature of the invention, the mixing procedure is begun near the maximum energy input which the drive can safely utilize, which is a function of the water/cement ratio on the decreasing portion of the curve, and the addition of water follows continuously with a corresponding continuous increase in the speed of the rotating elements of the mixer to maintain the energy input substantially constant.

Advantageously, according to a further feature of the invention, the maxing procedure is begun at an energy level approaching the maximum energy input to the mixer as a function of the water/cement ratio, and the remaining water is added in one portion with a simultaneous increase in the speed of the mixer in a single step. In this manner, a steep falling off of the curve of energy input versus water/cement ratio is avoided on addition of the remaining water. In this procedure, the number of revolutions is adjusted so that the drive motor of the mixer is operated at about its rated load in both mixing phases.

It has further been shown that the throughput of the above described preparation method can be increased by heating the concrete in the mixture. By heating, the strength of the early set concrete can be so increased that molds, frames and forms may be quickly removed from concrete bodies of large dimensions. For example, molds can be used three times within a twenty-four hour period. Such heating preferably takes place during mixing by the introduction of saturated steam at a pressure of 2.5-3 kg./cm.<sup>2</sup>, in a conventional manner. The temperature of the concrete should not exceed 60° C., however. For this embodiment, Portland blast-furnace cement is particularly suitable.

The mixing procedure may be carried out in a counter-current mixer with a main mixing system continuously rotating at uniform speed and a variable speed mixing element or agitator. When such countercurrent mixers are employed, the high speed mixing element strongly promotes the intensive preparation of mixed materials. In principle, it is possible to construct a mixer so that the rotative speed of the machine is adjustable over a wide limit, in which case the same machine can take over the function both of a mixing shovel and of a high speed mixing element. Mixing shovels are principally necessary for emptying the machine. By the use of a barrier wall it is possible to avoid the use of wide-area mixing shovels, so that all rotating systems can operate with a relatively high rate of speed and thereby noticeably increasing the overall effect.

A better understanding of the present invention will be had from the accompanying drawings in which FIG. 1 is a plot of several curves showing the energy requirement of a rotating type mixing element of a counter-current mixer at different speeds of rotation of the element and for mixtures of different consistencies;

FIG. 2 is a further plot of curves showing the continual increase in the speed of rotation of the mixing element with a continuous addition of water during the second process step of the present invention;

FIG. 3 is a schematic view of an apparatus suitable for carrying out the process of the invention;

FIG. 4 is a schematic plan view of the apparatus; and

FIG. 5 shows a drive mechanism for the mixing apparatus of FIGS. 3 and 4.

The curves of FIG. 1 were determined from using a counter-current mixer having a rotary mixing element and loaded with a mixture comprising 750 liters of aggregate, 175 kg. of cement, and 140 liters of water. The rotating element had the form of an H. Lower curve I was determined at an agitator revolution of 200 r.p.m., and upper curve II was determined at an agitator revolution of 400 r.p.m. Both curves clearly show the very different total energy input of the drive motor of the mixer for different numbers of revolutions and different consistencies of the mixture.

Curves I and II of FIG. 2 were plotted from data obtained from the same machine when filled with the same material as in FIG. 1. Upon reaching a nominal or rated load for the machine motor of about 40 kw. at point 1, the rotative speed of the [cyclone type] mixing element was continuously raised from 200 r.p.m. to 400 r.p.m. at point 2 with continuous addition of water until a desired water/cement ratio of 0.75 was reached. It can be seen from FIG. 2 that according to the process of the

invention the maximum energy input to the machine can be held at a substantially constant value, here shown as 40 kw., despite an increase in the rotative speed to 400 r.p.m. In contrast, if the same mixture of aggregate, cement, and water at a water/cement ratio of 0.75 was introduced initially into the machine and the rotating mixing element was run at a uniform speed of, for example, 400 r.p.m., during the entire mixing procedure, no intensive utilization of the mixing element in the preparation of the mixture or of the binder particles would be achieved because the mixture would not have the necessary consistency for energy intake. By operating in two steps, and during the first step only so much water is introduced as is necessary for wetting so that the water/cement ratio is in the region of about 0.3 to 0.4, a fine reduction of the binder is brought about from the very beginning and then is further increased in the second step of the process upon increasing the number of revolutions of the rotating mixing element and upon addition of the remaining quantity of water until the water/cement ratio is about 0.65, for example. Depending on the kind of mixture being worked, the first step of the intensive preparation requires only a very short period of time (for example 40-70 seconds), whereupon the addition of the remaining water follows and the number of revolutions of the rotating mixing element is increased. The latter is raised from time to time as the consistency of the mixture softens upon the addition of water, so that the drive motor is kept near its nominal or rated load. The mixture can be discharged after as little as an additional 20-40 seconds of operation.

The times given, by way of example, correspond to those usually encountered in practice. Nevertheless, it has been shown that longer mixing times are unusually economical if the highest possible savings in cement consumption are desired. Mixtures having a high proportion of cement are expensive merely because of their composition of raw ingredients. In the preparation of a concrete having 400 kg. of cement per cubic meter, for example, more grinding work must be expended than for a concrete having only 200 kg. of cement per cubic meter. According to the present process, the cost of the increased energy for additional mixing amounts on the average to only 3-5 percent of the resulting saving in cement, so that the increased expenditure of mechanical energy proves extraordinarily economical. The maintenance of the energy demand of the drive motor at a constant value is accomplished for different concrete formulations on the one hand by graduated water additions and, on the other hand, by varying of the speed of rotation of the mixing elements. It has been found that the energy demand of the drive motor for a rotating mixing element increases almost proportionally with the increase in the number of revolutions thereof, and that this ratio is variable within certain limits depending on the consistency of the material being mixed. Concrete mixtures having a low cement content, for example, show an almost constant, relatively high, specific energy demand over the entire range of consistencies conventional in concrete technology. Concrete mixtures having a high cement content, in contrast, have a steeply decreasing specific energy demand with increasing water/concrete ratio. With the addition of the remaining quantity of water required in one portion of the second process step together with a simultaneous discontinuous increase in the number of revolutions of the rotating mixing element, care must only be taken that the rated load of the drive motor for the mixing element is not exceeded. The advantages achieved in this embodiment correspond essentially with those of continual water addition and continual increase of the number of revolutions of the drive motor. In case of large variations in the moisture content of the concrete aggregate, the process of the invention can also be used for maintaining a certain constant concrete consistency, particularly when the consistency lies in the

region of the steeply decreasing branch of the energy requirement curve. In this case, the addition of water is stopped as soon as the energy input of the mixer has reached a value corresponding with the desired final consistency. Subsequently, the rotative speed of the mixing element is adjusted to the maximum permissible load and the intensive preparation is completed. For the preparation of very soft mixtures, a first quantity of water can be added depending on machine load, that is, the addition of water is discontinued when a value in the neighborhood of the energy maximum is reached. At the conclusion of the intensive mixing, any residual portions of water still lacking can be quickly introduced with a water meter and the mixing continued, or the step of adding the remaining water may be eliminated if the smaller drive demand corresponding with the desired region of consistency is reached.

Variable speed electric or hydraulic motors can be employed to drive the mixing element. Regulation of the rotative speed can be carried out by means of automatic control switches either automatically or by hand.

#### Example I

An aggregate having a particle size of from 0-30 mm. and a suitable amount of cement, for example in a ratio of 3400 kg. aggregate to 500 kg. cement, is supplied to a countercurrent mixer having a mixing apparatus and a cyclone type mixing element. Water is then added as quickly as possible in an amount such that the drive motor is loaded to its full rated load. In practice, a wattmeter will initially indicate that the energy input exceeds the rated load of the motor during the course of water addition. So much additional water then must be added that the watt meter returns to the rated load for the motor. For this composition, intensive mixing takes about a minute. However, the duration of the intensive mixing is dependent on the amount of cement employed and for larger quantities of cement, a longer intensive mixing is necessary in order to achieve fine reduction of the numerous particles. Prior test runs are used to determine which specific power consumption and in which time the optimum cement yield can be obtained, that is, the most satisfactory relationship between early strength, final strength and ease of workability for a particular concrete composition. After conclusion of this intensive mixing, the remaining amount of water is added in order to bring the concrete to the desired consistency, and then the mixture is removed from the mixer.

#### Example 2

Cement, sand, and gravel are introduced as dry components into a countercurrent mixture as above and the total quantity of water desired for the final consistency is added. The variable speed mixer element or elements are then set at such an r.p.m. rate that the rated load of the drive motors is reached. Mixing is continued at rated load by varying the speed of rotation of the rotary mixing element or elements until the optimum binder utilization has been achieved, as determined by prior exploratory tests. This is in distinction to the mixing techniques heretofore used in the art where the mixing machine always operates at the same rotative speed independent of the consistency and of the kind of concrete being prepared. Nevertheless, even in the preparation of concrete of a relatively soft consistency, the amount of energy necessary for an intensive preparation are not used.

For an economic intensive preparation or mixing, it is of decisive significance that the machines used operate at full load capacity during the entire preparation process, even when the material being handled has sharply varying properties. Overloading and partial loading should not result because of the transitions between regions of different consistency required according to the present process. For this reason, a regulation of the speed of rotation depending on load is necessary. For example, hydraulic drives can be used. This kind of drive is rela-

tively expensive, since a pump and an hydraulic motor controllable over a wide r.p.m. range, together with the accompanying expensive oil supply regulation, are necessary in addition to an electric motor. Remotely controlled variable speed regulators also can be employed in principle. For the loads in question these are not only very expensive, but also cause difficulties with installation because of their dimensions. Direct current special motors also can be adjusted over a wide r.p.i. range. They also are relatively expensive in contrast with alternative motors and, in addition to the direct current motor, a direct current generator must be used. Pole changing motors have a control region which is too small for intensive preparation or mixing of the invention in general, or, in other words, for good utilization of the apparatus which requires a control region of about 1:10. Variable alternating current motors do develop good torque characteristics as soon as the desired number of revolutions is reached. On the other hand, these motors in their standard form have the disadvantage of not being able to accelerate under a heavy load from a low to a high rotative speed.

Proceeding from these considerations, a relatively simple drive apparatus, shown in FIGS. 3-5, has been developed to meet the demands of an intensive preparation according to the invention. The apparatus consists essentially of a mixing bowl 1, which from the point of view of its construction and drive corresponds with the disc of a countercurrent mixer, and having a closure disc 2 for a discharge opening, a high speed mixing element 3 which operates to produce mixing, and a movable emptying blade 4 positioned as shown in full lines when the discharge opening is open, and, during the mixing procedure, being either in the position shown in dotted lines in FIG. 3 or lifted above the material being mixed, or in the concentric position shown in dotted lines in FIG. 4. As shown by the arrows in FIG. 4, the mixing bowl 1 may be rotated in a clockwise direction by conventional mechanism not shown in the drawings and the high speed mixing element 3 may be rotated in a counter-clockwise direction by mechanism described hereafter. Positioning rod 5 is either movable vertically (FIG. 3) or rotatable within a limited angle (FIG. 4).

The drive for the drive shaft 6 of the rotating mixing element 3 is shown in FIG. 5. An electric motor 7, operable in at least two speeds, drives a V-grooved pulley 8 or a gear wheel at a corresponding ratio, for example 4:1 or 5:1. On each of its upper and lower faces, pulley 8 carries clutch discs 9 and 10, each of which is provided with a clutch facing. The opposing clutch halves each have a pinion 11 and 12 linked to shaft 6 of the mixing element in a ratio of 1:1 or 1:4 (or 1:5). The clutch discs are positioned on a stationary shaft 13 which is, however, vertically moveable. If the machine is to run at the lowest speed, the drive motor is started and brought up to a high speed of, for example, 1500 r.p.m. Then shaft 13 carrying the clutch discs is lifted and clutch 10 is brought into engagement. In analogous fashion, the upper coupling half 9 is activated. The shifting of the clutch can take place manually, or by electric motor, through a small worm and wheel drive with limit switching. Continual contact pressure and maintenance of the median position is achieved by means of a spring introduced into the vertically moveable arrangement. Starting and switching of the drive motor follows from time to time from the idling position with the clutch in an intermediate position. All gears remain in mesh. It is possible to change the direction of rotation if desired.

The emptying blade 4 illustrated in the drawings can be omitted in mixers having bowls which can be tipped for emptying.

The curves of FIGS. 1 and 2 and the working examples pertain to mixtures containing cement. However, the invention is also applicable to materials containing lime as a binder, for example calcium silicate brick (sandlime brick) mixtures. In the latter, the avoidance of binder aggregates and the promotion of sand abrasion are critical

because the presence of sufficiently fine quartz powder is necessary for the development of the binding strength of the lime.

According to the process of the invention, a higher initial strength is obtained as the final result but, in many cases, an increase in final strength and an improvement in workability are also achieved. Also, in many cases the smoothing of the particle surfaces brought about by intensive mixing is an advantage, because rough particle surfaces lead to an increase in consumption in water and cement without any increase in compressive strength.

We claim:

1. A process for the intensive mixing of the ingredients of a construction material with the aid of a mixing apparatus having at least one variable speed mixing element and a power operated drive for the mixing element, which comprises the steps of supplying an aggregate, binder and thinner to the apparatus, adding thinner to the apparatus for varying the consistency of the mass, rotating the mixing element at different speeds in the materials supplied to the apparatus to mix the materials at the rated capacity of the drive, and varying at least one of the steps consisting of varying the speed of the mixing elements and adding thinner to the apparatus so as to maintain the energy input substantially constant at the rated capacity of the power operated drive for at least the time required to produce a homogeneous mixture, thereby to produce a more intensive utilization of the mixing apparatus.

2. A process in accordance with claim 1 in which the binder is cement, the thinner is water and the mixing is continued until no increase in the quality of mixed product can be obtained.

3. A process in accordance with claim 2 in which the water and binder ratio initially supplied requires an energy input near the maximum capacity of the power operated drive.

4. A process in accordance with claim 2 in which only a portion of the total amount of water required is initially supplied to maintain the energy input at the rated capacity of the drive, subsequently adding the additional water required, and simultaneously increasing the rotational speed of the mixing element so as to maintain substantially the same energy input to the mixing element.

5. A process in accordance with claim 4 in which all of the additional water required is added at one time and the corresponding increase in speed of rotation of the mixing element is produced in one step.

6. A process in accordance with claim 4 in which the additional water is gradually added and the speed of rotation of the mixing element is gradually increased.

7. A process in accordance with claim 2 in which the materials are heated to a temperature not exceeding 60° by the addition of saturated steam as they are being intensively mixed.

8. A process in accordance with claim 1 in which the mixer has a mixing element rotatable in one direction to act on the material during mixing, and a variable speed rotating element rotatable in a countercurrent direction to said first mentioned element.

#### References Cited

##### UNITED STATES PATENTS

|           |         |                      |
|-----------|---------|----------------------|
| 3,062,514 | 11/1962 | Waimer.              |
| 3,081,983 | 3/1963  | Thibodeaux.          |
| 3,160,400 | 12/1964 | Harrison.            |
| 3,326,535 | 6/1967  | Clerex ----- 259—147 |

ROBERT W. JENKINS, Primary Examiner

U.S. Cl. X.R.

35 259—85, 177